

## 1

3,580,722

### LIGHT-SENSITIVE SILVER HALIDE COLOR PHOTOGRAPHIC EMULSION

Kenro Sakamoto, Takao Takahashi, Takeo Koitabashi,  
and Mitsuto Fujiwara, Tokyo, Japan, assignors to  
Konishiroku Photo Industry Co., Ltd., Tokyo, Japan  
No Drawing. Filed Feb. 6, 1969, Ser. No. 797,277  
Claims priority, application Japan, Feb. 9, 1968,  
43/7,748

Int. Cl. G03c 1/40

U.S. Cl. 96—100

6 Claims

#### ABSTRACT OF THE DISCLOSURE

A color photographic emulsion containing a color former of the formula:



and at least one compound of the formula:



or



wherein R1 is alkyl, acylamino or sulfonamido; X1, X2 and X3 are hydrogen, alkyl, halogen, acylamino, alkylcarbamoyl, sulfonamido, sulfamoyl, alkoxy or aryloxy; A and B are —COR2, —COOR2', —CONHR2'' or —CN; R2, R2', R2'', X4 and X5 are allyl, alkyl, aryl, cycloalkyl or aralkyl and F is an atom or radical necessary to form a pyrazolone ring.

This invention relates to a light-sensitive silver halide color photographic emulsion capable of forming a color image by color development. In particular, the invention relates to a color photographic emulsion containing a pyrazolone derivative as a magenta color former.

More particularly, the color photographic emulsion contains at least one of the color formers of the general Formula I and at least one of the compounds of the general Formulas II and III.



## 2

In the above formulas.

R1 is an unsubstituted or substituted alkyl, acylamino or sulfonamido group;

X1, X2 and X3 which may be the same or different are hydrogen, unsubstituted or substituted alkyl, halogen, acylamino, unsubstituted or substituted alkylcarbamoyl, sulfonamido, unsubstituted or substituted sulfamoyl, alkoxy or aryloxy group;

A and B are —COR2, —COOR2', —CONHR2'' or —CN; R2, R2', R2'', X4 and X5 are substituted or unsubstituted allyl, alkyl, aryl, cycloalkyl or aralkyl groups; and F represents an atom or radical necessary for forming a pyrazolone ring.

As the result of various investigations on the silver halide photographic emulsions containing a color former, it is known that a light-sensitive photographic material prepared from a silver halide photographic emulsion containing only a color former with low coupling reactivity,

when treated by a developing solution consisting principally of a p-phenylenediamine derivative, readily produces a linear gradation, but the speed of development is delayed on account of low coupling reactivity and the density is insufficient. Consequently the contrast of the resulting

image is low and sufficient photographic sensitivity is not obtainable. In order to overcome the above disadvantages, it has been proposed to increase the quantity of the color former and silver halide or to increase the thickness of the emulsion layer. As is well known, however, both of the

above improvements have serious drawbacks and the disadvantages as aforementioned cannot satisfactorily be solved thereby. More particularly, an increase in the quantity of the color former and silver halide results in a considerable increase in viscosity of the emulsion and coating

of such emulsion on a support is difficult. Further, such an emulsion is very readily fogged and is inferior in stability of photographic properties. On the other hand, an increase in the thickness of the emulsion layer results in depression of the sharpness of the resulting images on account of halation, inadication and other factors.

Under the circumstances, a combination comprising a color former showing low coupling reactivity and a color former showing relatively high coupling reactivity has been proposed. The drawbacks of the aforementioned

prior processes are somewhat improved with said combination. However, mixing of the developed dyes is caused by the combination of two or more of the different color formers so that an undesirable color shift occurs. This makes it impossible to use the emulsion for color photography, consequently.

Now, according to the present invention, it has been found that at least one of the color formers of the above general Formula I which shows low coupling reactivity is added to a silver halide photographic emulsion in combination with at least one of the compounds of the general Formulas II and III which reacts with an oxidation product of p-phenylenediamine derivative to form a colorless coupling product. The resulting emulsion does not suffer from any change of spectral absorption characteristic of the developed dyes and, what is more, the speed and gamma values are extremely increased.

Thus, according to the silver halide color photographic emulsion having increased speed and gamma values of this invention, a small amount of the color former is sufficient and the viscosity of the emulsion is decreased and consequently, coating of the emulsion on a support can easily be made. Further, such an emulsion is safe from fogging and the thickness of the emulsion layer is reduced. With such an emulsion, a light-sensitive color photographic material having improved sharpness of the resulting image may be obtained.



Typical color formers of the general Formula I are as follows:



Typical compounds of the general Formula II are as follows:



3,580,722



Typical compounds of the general Formula III are as follows: 25



It should be understood that the color former of the general Formula I and the compounds of the general Formulas II and III used in this invention are not limited to those exemplified above, and alkali metal salts or ammonium salts of the sulfonic acid or carboxylic acid of the general Formulas I and II or III are included within the scope of the present invention.

65      Addition of at least one color former of the general Formula I and at least one of the compounds of the general Formulas II and III to the photographic emulsion may be made either directly in the form of an aqueous alkali solution such as sodium hydroxide or in the form  
70      of a dispersion prepared by dissolving the color former of the general Formula I and the compounds of general Formulas II, III in a low boiling organic solvent such as butyl alcohol and butyl acetate and a high boiling organic solvent such as dibutyl phthalate, mixing the resulting solution with a gelatine solution containing a  
75

surface active agent and then treating the mixture in a colloid mill. Alternatively, addition may be made by means of a known dispersion method. Each of the compounds of the general Formulas II and III is used in a molar ratio of 0.05-1 to the color former of the general Formula I, particularly a molar ratio in the range of 0.1-0.5 is effective.

For the photographic emulsion of the present invention, various silver halide emulsions such as silver chloride-, silver bromide-, silver iodide- and silver chlorobromide emulsions are usable and these emulsions may further contain a chemical sensitizer such as sulfur-, reduction-, or noble metal-sensitizer and an optical sensitizer and, in addition, various additives, for example, a fog inhibitor, a stabilizer, an anti-stain agent, a developing accelerator, a hardening agent and a coating aid, etc.

Further, when optically sensitized emulsions are coated in the same place in two layers, the color former of the general Formula I and the compounds of the general Formulas I and II are applicable to either or both of such emulsions.

This invention will be explained in more detail by the following examples wherein all parts given are by weight:

#### EXAMPLE 1

To 100 parts of a light-sensitive gelatino silver bromoiodide emulsion prepared by a conventional manner and containing a green sensitive optical sensitizer are added, a 5% aqueous alkali solution of the color former (I-7) and a 5% aqueous alkali solution of the compound (III-2) or (III-4) in the amounts indicated in the Table 1 below. The thus treated emulsion is coated on a film base. The resulting film is then treated at 20° C. for 10 minutes with a developing solution comprising as the principal color developer N,N-diethyl-p-phenylenediamine and thereafter subjected to bleaching and fixing. Increase of the density is shown in Table 1 by way of the photographic gamma value measured by using green light density. The emulsions of this invention exhibit remarkable increases in gamma values.

TABLE 1

| Color former I | Compound III | Gamma |
|----------------|--------------|-------|
| I-7 (21)       | III-2 (0)    | 0.29  |
| I-7 (21.5)     | III-2 (0)    | 0.30  |
| I-7 (22)       | III-2 (0)    | 0.32  |
| I-7 (20)       | III-2 (1)    | 0.36  |
| I-7 (20)       | III-2 (1.5)  | 0.39  |
| I-7 (20)       | III-2 (2)    | 0.53  |
| I-7 (20)       | III-4 (1)    | 0.33  |
| I-7 (20)       | III-4 (1.5)  | 0.37  |
| I-7 (20)       | III-4 (2)    | 0.51  |

NOTE.—Figures in parentheses are parts.

#### EXAMPLE 2

A similar film is prepared in the same manner as in Example 1 by using a 5% aqueous alkali solution of the color former (I-7) and a 5% aqueous alkali solution of compound (III-1) in the amounts indicated in the Table 2 below, respectively. The resulting film is then treated in the same manner as in Example 1. Gamma values as measured are shown in Table 2. As is obvious from Table 2, the emulsions of this invention exhibit remarkable increases in gamma values.

TABLE 2

| Color former I | Compound III | Gamma |
|----------------|--------------|-------|
| I-7 (21)       | III-1 (0)    | 0.36  |
| I-7 (21.5)     | III-1 (0)    | 0.38  |
| I-7 (22)       | III-1 (0)    | 0.40  |
| I-7 (20)       | III-1 (1)    | 0.46  |
| I-7 (20)       | III-1 (1.5)  | 0.50  |
| I-7 (20)       | III-1 (2)    | 0.68  |

NOTE.—Figures in parentheses are parts.

#### EXAMPLE 3

Three mixtures, each comprising 1 part of the color former (I-8) and 1, 1.5 or 2 parts of the compound

(III-5), respectively, are separately dissolved in 3 parts of ethyl acetate by heating. Each of the resulting solutions is added with 1 part of dibutyl phthalate. The solution thus obtained is then mixed with 10 parts of an aqueous 10% gelatine solution and passed through a colloid mill to form the color former dispersion. The same amount of this dispersion as that used in Example 1 is added to an emulsion containing an adjusted amount of gelatine to give the same gelatine content as of Example 1 in the finished total emulsion. Photographic gamma values observed with a film prepared and treated in a similar manner to that in Example 1 are shown in Table 3.

TABLE 3

| Color former I | Compound III | Gamma |
|----------------|--------------|-------|
| I-8 (21)       | III-5 (0)    | 0.30  |
| I-8 (21.5)     | III-5 (0)    | 0.31  |
| I-8 (22)       | III-5 (0)    | 0.33  |
| I-8 (20)       | III-5 (1)    | 0.37  |
| I-8 (20)       | III-5 (1.5)  | 0.42  |
| I-8 (20)       | III-5 (2)    | 0.57  |

NOTE.—Figures in parentheses are parts.

As is obvious from Table 3, the emulsions of this invention have remarkably increased gamma values.

#### EXAMPLE 4

A similar emulsion as used in Example 1 is prepared by adding a 5% aqueous alkali solution of the color former (I-7) and a 5% aqueous alkali solution of the compound (II-1) each in the amounts indicated in Table 4, in which photographic gamma values observed with a film prepared and treated in a similar manner to that in Example 1 are shown.

TABLE 4

| Color former I | Compound III | Gamma |
|----------------|--------------|-------|
| I-7 (21)       | II-1 (0)     | 0.26  |
| I-7 (21.5)     | II-1 (0)     | 0.27  |
| I-7 (22)       | II-1 (0)     | 0.28  |
| I-7 (20)       | II-1 (1)     | 0.30  |
| I-7 (20)       | II-1 (1.5)   | 0.33  |
| I-7 (20)       | II-1 (2)     | 0.37  |

NOTE.—Figures in parentheses are parts.

As is obvious from the above table, the emulsions of this invention have outstandingly increased gamma values.

#### EXAMPLE 5

A similar emulsion as used in Example 1 is prepared by adding a 5% aqueous alkali solution of the color former (I-7) and a 5% aqueous alkali solution of the compound (II-5) each in the amounts indicated in Table 5, in which photographic gamma values observed with a film prepared and treated in the same manner as in Example 1 are shown.

TABLE 5

| Color former I | Compound III | Gamma |
|----------------|--------------|-------|
| I-7 (21)       | II-5 (0)     | 0.17  |
| I-7 (22)       | II-5 (0)     | 0.18  |
| I-7 (23)       | II-5 (0)     | 0.20  |
| I-7 (20)       | II-5 (1)     | 0.22  |
| I-7 (20)       | II-5 (3)     | 0.24  |
| I-7 (20)       | II-5 (5)     | 0.27  |

NOTE.—Figures in parentheses are parts.

In the above examples, the present invention is illustrated as to the case where the combination of one of the color former and one of the other compound is used but it has been observed that the same effects are obtainable by using the combination of, for example, the color former (I-1) and the compounds (III-1) and (III-2).

What is claimed is:

1. A silver halide color photographic emulsion comprising at least one color former of the general Formula

92

I together with at least one of the compounds of the general Formulas II and III;



wherein,

$R_1$  represents an alkyl, acylamino or sulfonamido group;  $X_1$ ,  $X_2$  and  $X_3$  which are same or different represent hydrogen, an alkyl, halogen, acylamino, alkylcarbamoyl, sulfonamido, sulfamoyl, alkoxy or aryloxy group;

A and B represent  $-\text{COR}_2$ ,  $-\text{COOR}_2'$ ,  $-\text{CONHR}_2''$  or  $-\text{CN}$ : 25

$R_2$ ,  $R_2'$ ,  $R_2''$ ,  $X_4$  and  $X_5$  represent allyl, alkyl, aryl, cycloalkyl or aralkyl group;  
 $F$  represents an atom or radical necessary to form a pyrrole ring.

2. A silver halide color photographic emulsion as claimed in claim 1, comprising the color former of the formula



in combination with a compound of the formula,



οι



3. A silver halide color photographic emulsion as claimed in claim 1, comprising the color former of the

10

Formula I-7 in combination with the compound of the formula,



5

[III] 4. A silver halide color photographic emulsion as claimed in claim 1, comprising the color former of the formula,



in combination with the compound of the formula,



5. A silver halide color photographic emulsion as claimed in claim 1, comprising the color former of the Formula I-7 in combination with the compound of the formula,



50 6. A silver halide color photographic emulsion as claimed in claim 1, comprising the color former of the Formula I-7 in combination with the compound of the formula



## References Cited

## FOREIGN PATENTS

721,520 1/1955 Great Britain ----- 96-100

J. TRAVIS BROWN, Primary Examiner

U.S. Cl.X.R.

96-107